

## UNITED STATES PATENT OFFICE

JOHN WESLEY MARDEN AND HARVEY CLAYTON RENTSCHLER, OF EAST ORANGE, NEW JERSEY, ASSIGNEES TO WESTINGHOUSE LAMP COMPANY, A CORPORATION OF PENNSYLVANIA

## ELECTRON-EMISSION MATERIAL

No Drawing.

Application filed March 8, 1926. Serial No. 93,308.

This invention relates to electron-emitting cathodes and more particularly to a cathode comprising a refractory metal body having incorporated or deposited thereon, material having high electron-emitting properties.

One of the objects of this invention is to provide a material of the above nature having high electron-emission and which will maintain such emission under adverse conditions for a long commercial life.

Another object is to provide an electron-emitting material, the emission of which may be readily restored should the same be impaired or destroyed.

Other objects and advantages will appear as the description proceeds.

The present invention is based on the discovery that vanadium when incorporated in small percentages in refractory metals, such as tungsten, molybdenum, tantalum, etc., or coated thereon imparts to the metal body a high emission comparable with that obtained with thorium under similar conditions. Vanadium, however, as an electron-emitting material, has certain advantages over thorium as will hereinafter more fully appear.

Heretofore thorium has been considered one of the most practical of electron-emitting materials. It is readily worked into tungsten in small percentages and has a high electron emission at a moderate temperature at which temperature the rate of evaporation is very low. In producing thoriated tungsten wire for electron emission purposes

it is usual to introduce the thorium into the wire in the form of thorium oxide since it is difficult to prevent thorium metal from volatilizing out at the temperatures to which the material is subjected during manufacture. The thorium oxide is later reduced to thorium metal. One method largely used for obtaining this reduction of thorium oxide is to flash the filament in a hydrocarbon atmosphere such as described in application

Serial No. 636,510 of Ralph E. Myers, filed May 3, 1923, entitled Evacuated devices and method of exhaust, and assigned to the Westinghouse Lamp Company.

Another process is that described in application Serial No. 620,485 of John W.

Marden et al., filed February 21, 1923, entitled Activation of electron-emission material, and assigned to the Westinghouse Lamp Company.

In this latter method the thorium is introduced into the filament in the form of thorium carbide. In both of the above methods it is believed that thorium carbide is ultimately formed, which after the filament is sealed in the envelope and the same exhausted, is decomposed by heating the filament to a high temperature. While such process produces material of high electron-emitting properties it is somewhat involved and requires careful supervision. Difficulty has also been experienced when employing thoriated cathodes in maintaining the thorium emission for a considerable period of time due to oxidation of the thorium by minute quantities of oxygen liberated from the electrodes. This is particularly true in low power tubes such as the usual dry cell tubes employing a short filament having a very limited quantity of thorium metal available for electron emission. In order to prevent this oxidation of the thorium it is the usual practice to bake out the anode plates and grids in hydrogen before sealing-in in order to remove all oxygen therefrom and after completion of the tube to heat the plate by high frequency induction current to a high temperature, i. e., around 900 to 1000° to drive out all occluded gases and vaporize the metallic clean-up agent therefrom.

In spite of these precautions, however, an oxide film persists on the surface of the plate which is subsequently decomposed by electron bombardment from the cathode during operation of the device, with the liberation of oxygen which migrates to the filament and oxidizes the thorium film thereon destroying its emission. The thorium oxide so formed cannot be reduced again and the emission of the filament is permanently impaired.

It is one of the aims of the present invention to avoid the difficulties inherent in the use of thorium activated cathodes and to provide an electron-emitting material, the emission of which may be readily developed

and maintained or if impaired may be readily restored.

We have observed when treating vanadium at high temperature in a high vacuum that near the melting point of the vanadium it has a very low vapor pressure and does not volatilize to any extent. We have also discovered that at such temperatures vanadium has an extremely high electron emission and when incorporated into a carrier metal such as molybdenum in small percentages, that it imparts to the metal body substantially the same emission as if the body were composed entirely of vanadium.

It has been proposed heretofore to produce a tungsten filament containing thorium, vanadium, yttrium oxide and a number of other materials. Such a product is disclosed in the patent to Laise 1,569,095. The method of producing such a wire is extremely involved and laborious. The vanadium which is added to the wire in addition to the thorium and other materials is ineffective to increase or augment the electron emission of the thorium under the existing theories of electron emission from thoriated cathodes. It is generally accepted that the thorium forms a film on the surface of the filament, one atom deep and that any surplus thorium rapidly vaporizes away. If the entire filament is thus covered with an atom deep layer of thorium the filament will have its maximum emission and the addition of vanadium to the filament will not increase this emission. If a portion of the surface layer of thorium is replaced by vanadium the electron emission of the filament as a whole will be decreased slightly since the emission of vanadium is slightly less than that of thorium. It is obviously impossible to determine in a filament containing both thorium and vanadium how much emission is due to the presence of thorium and how much is due to vanadium.

The present applicants have found that it is unnecessary to employ the involved process, such as disclosed in the Laise patent, or to include in the filament the many different materials specified by him. Electron-emitting filaments having properties substantially equal to those of thorium activated cathodes and in addition being free from the objections specified above may be readily produced by the usual processes of producing tungsten, molybdenum and tantalum which are highly developed and greatly simplified. In order to produce a molybdenum filament containing vanadium, for instance, it is only necessary to mix the powdered molybdenum or molybdenum oxide with a vanadium compound, such as ammonium vanadate, reduce the same in hydrogen, press the powdered material into slugs and sinter, swage and draw the same in the manner well known in the art for producing molybdenum filaments.

The proportion of vanadium required in the completed wire is very small, excellent results having been obtained with wire containing less than .5% of vanadium metal. Preferably, sufficiently finely divided vanadium or reducible vanadium compound such as ammonium vanadate or vanadyl sulphate or nitrate should be added to the refractory metal powder to produce, after reduction, from .5 to 1% of vanadium. Larger percentages do not appreciably augment the emission and render the wire more difficult to work. Caution should be observed during the various heat treatments to which the material is subjected during fabrication to treat the wire at as low a temperature as is consistent with proper mechanical working of the body in order to avoid distillation of the vanadium from the metal. When employing tungsten as the base or carrier metal, heating the wire to high temperatures in hydrogen should be avoided since hydrogen has a strong tendency to embrittle the same. Such brittleness, however, may be readily removed by subjecting the wire to an anodic treatment in a caustic soda solution such as that described and claimed in a copending application of Malcolm N. Rich, Serial No. 4140, filed January 23, 1925, entitled Pliable tungsten and method of producing the same and assigned to the Westinghouse Lamp Company. When the vanadium is incorporated into tantalum filaments such wires may be fabricated by the cold working process well known in the art for producing tantalum wire.

As a specific example of the production of vanadium activated cathodes, vanadyl nitrate was added to finely powdered molybdenum in sufficient quantity to produce .625% of vanadium metal to molybdenum metal. The mixture was reduced in a stream of hydrogen in the usual manner, the temperature being maintained at about 1000° C. for a period of several hours in order to insure complete reduction. The reduced mixture was then sieved and pressed into a slug of one-quarter inch cross section. The slug was sintered and treated in hydrogen by passing the current therethrough sufficient to heat the same to about 80% of its fusing temperature. In the case of the one-quarter inch slug a current of 920 amperes was required for obtaining the desired heat. The slug was then swaged to 36 mil size in the usual manner and drawn to final size, annealing being resorted to at the 14 mil size to remove work hardening effects and recrystallize the wire so that the further drawing could be accomplished.

While vanadium activated molybdenum has been cited by way of specific example it is to be understood that the vanadium may be readily incorporated into other metals, such as tungsten and tantalum in accordance

with the well known methods for producing such metals.

We have found that the vanadium activated filaments, when enclosed in an evacuated container, have a high emission at moderate temperatures and that such emission may be maintained for a long period of time without diminution. By way of comparison several tests were made on electron tubes employing thorium activated and vanadium activated cathodes. In the case of the thorium activated cathode tubes it was found that the emission was quite constant at plate potentials around 50 volts but that when the voltage was raised to 70 volts there was a decided loss in emission, the emission dropping from approximately 50 milliamperes to 20 milliamperes in about 40 minutes. This is explained on the theory that at higher plate voltages the electron bombardment of the plate was sufficient to decompose the oxide film which is always present there, liberating oxygen which oxidized the thorium impairing the emission of the cathode. In the case of vanadium activated filaments under similar treatment, the emission dropped only from 48 milliamperes to 38 milliamperes, or about one-third of the loss of emission which was experienced with the thoriated cathode. This property of vanadium activated filament of resisting loss of emission by oxidation is due to the property of vanadium oxide of decomposing below the temperature at which the filament is normally operated and is of extreme value since it permits of the use of high plate current, which heretofore in the commercial production of electron devices has caused great difficulty due to the oxidation of the thorium on initial operation of the device.

The vanadium activated filaments, moreover, were found to regain their emission much more readily than did the thorium activated cathodes due to the property of the vanadium oxide of being decomposed by heat alone. In the case of the vanadium doped filaments it is only necessary when this emission is impaired by oxidation to elevate the temperature of the cathode slightly in excess of its normal operating temperature in order to reduce the vanadium oxide and restore the original high emission of the filament. In the test referred to above, the plate voltages were raised to 100 volts and further loss in emission in both filaments experienced. The filaments were then reseasoned to restore the emission and after such treatment the vanadium activated filament gave an emission much in excess of that of the thorium activated filament, indicating clearly that the vanadium is much more resistant to the abuse to which electron devices may be subjected in use than are thoriated cathodes and while their initial emission may be slightly less than that of thorium, the in-

dications are that in the commercial production of tubes, after seasoning, the vanadium activated filaments will have a higher emission and longer life than thorium activated cathodes.

While the vanadium is preferably incorporated into the cathode as an alloy or mixture with the carrier metal, if desired it may be coated thereon or employed in various other manners for electron emission purposes. Obviously, various other modifications and changes may be made in the invention described without departing therefrom.

What is claimed is:

1. In an electron discharge device utilizing a thermionically active cathode and at least one cooperating electrode, a cathode comprised of a refractory metal base containing approximately 1.0 per cent of vanadium.

2. In an electron discharge device utilizing a thermionically active cathode and at least one cooperating electrode, a cathode comprised of molybdenum containing approximately 1.0 per cent of vanadium.

In testimony whereof, we have hereunto subscribed our names this 5th day of March, 1926.

JOHN WESLEY MARDEN.  
HARVEY CLAYTON RENTSCHLER.

95

100

105

110

115

120

125